

## UNITED STATES PATENT OFFICE

2,332,047

PROCESS OF PREPARING NITROGENOUS  
CELLULOSE DERIVATIVES

Louis H. Bock, Glenside, and Alva L. Houk, Philadelphia, Pa., assignors to Röhm &amp; Haas Company, Philadelphia, Pa.

No Drawing. Application October 21, 1939,  
Serial No. 300,654

6 Claims. (Cl. 8—124)

This invention relates to the treatment of cellulosic fibers, yarns, and fabrics with aminomethylene amino-1,3,5-triazines in order to impart to the cellulosic materials improved properties. In particular, it deals with imparting to cellulose permanently improved properties as shown by the handle, feel, appearance, and resistance to water of the treated material, decreased shrinkage on wetting and by the capacity of the treated cellulosic material to take up and hold dyestuffs which ordinarily are of value only with wool and silk.

Although many processes have been suggested for "animalizing" cellulose fibers, they have lacked the simplicity and economy essential for practical application or have brought about such changes in the fibers that they were no longer suitable for the purposes originally intended and that the fundamental advantages of cellulose fibers have been lost. We have found, furthermore, that many types of nitrogen linkage which have been added to cellulose are not truly effective for the "animalizing" of cellulose. Nor is the coating of cellulose with nitrogenous resins truly effective in accomplishing our objects.

It is the object of this invention to form nitrogenous derivatives of cellulose which improve the usual properties thereof. It is an object to impart to cellulose fibers a desirable finish as to softness, suppleness, resistance to water, resistance to shrinkage, and affinity for dyes ordinarily used only for wool and silk. It is an object to provide a simple, practical process for accomplishing the desired modification of cellulose. It is an object to produce permanent modifications of cellulose. It is an object to provide a method for "animalizing" cellulose which may be accomplished in the ordinary course of textile manufacture and which utilizes equipment commonly found in textile mills.

We have found that cellulose is readily reacted with aminomethylene amino-1,3,5-triazines and that by the proper choice of substituents in the triazine group a wide range of effects may be produced. Thus the cellulose may be rendered moderately soft or given a full, pleasing hand. If long chain derivatives are selected, water-proof or water-resistant effects are obtained. Cellulose treated with aminotriazines becomes markedly receptive to dyes ordinarily used only with wool and silk. We have found that the type of nitrogen linkages imparted in this process is unusually effective in "animalizing" cellulose. The treatment may be given only to the surface of the cellulosic material, particularly when dilute solutions are

5 applied, or by thorough impregnation with the treating solution the cellulose may become in relatively large part converted to an organic substitution derivative of cellulose containing a methylene amino-1,3,5-triazine group.

As cellulosic materials there may be used cotton, linen, jute, hemp, or other natural fibers of cellulose, or the cellulosic materials prepared from cotton, linters, wood cellulose, or the like by solution and regeneration and which are particularly improved by the treatment herein described. Mercerized cotton and linen, hydrated cellulose, cellulose ethers, and cellulose esters, in short any type of water-insoluble cellulosic material possessing hydroxyl groups, may be treated by our process. The cellulose may be in the form of fabrics, fibers, yarns, battings, sheets, or strips and may be fibrous or non-fibrous.

20 The aminomethylene amino-1,3,5-triazines, used for treating cellulose, are prepared by reacting an amino-1,3,5-triazine with formaldehyde and a non-aromatic monoamine possessing a hydrogen atom attached to the nitrogen. The preparation of such condensates is described in detail 25 in our copending application Serial No. 300,548 filed October 21, 1939, which on August 6, 1940, issued as United States Patent No. 2,210,831. There may be reacted at least one mol each of 30 formaldehyde and the amine for each mol of an amino-1,3,5-triazine, and as many as three to six mols of each may be reacted with a mol of a triazine possessing a like number of positions available for substitution. Aminomethylene derivatives may be obtained from ammelide, ammeline, melamine and any of their derivatives 35 containing an amino group, representative examples of which are the diacyl ammelines, such as distearyl ammeline, the preparation of which is described in our copending application Serial 40 No. 300,549 filed October 21, 1939, which on February 17, 1942, issued as U. S. Patent No. 2,273,687, or the 2-alkyl, 4-amino-6 hydroxy-1,3,5-triazines, and similar compounds in which the triazine group carries an aliphatic, aromatic, 45 aralkyl, alicyclic, or heterocyclic substituent, or a halogen, cyano group, or other group such as 1-cyano-2-amino-4,6-dimethyl-1,3,5-triazine or 2-chloro-4,6-diamino-1,3,5-triazine, or from tautomers of such compounds.

50 The preferred aminotriazine derivatives are those synthesized from one molar proportion of an amino-1,3,5-triazine and at least one mol each of formaldehyde in any of its various forms and an amine having at least one hydrogen atom attached to the amine nitrogen atom and posses-

sing no substituent group of over eight carbon atoms, since this amino group is split out in the reaction of an aminomethylene amino-1,3,5-triazine with cellulose. The most satisfactory derivatives are those prepared from non-aromatic, strongly basic, secondary amines.

Typical amines which may be used include monomethylamine, dimethylamine, monobutylamine, diethylamine, diallylamine, benzylamine, cyclohexylamine, morpholine, piperidine, pyrrolidine, etc.

In the application of the aminomethylene derivatives of the amino-1,3,5-triazines to cellulose, the usual procedure requires solution or dispersion of the desired compound in a treating bath. The compounds of relatively small molecular size are soluble directly and those with larger substituents usually disperse easily. In the case, however, of highly substituted or long chain derivatives solubility may be improved by the use of acids, such as acetic, formic, hydrochloric, etc. which form salts with the amino groups. The solutions or dispersions are stable and may be applied cold or hot, as desired. The presence of acids or salts of a strong acid and weak base seems to aid in the reaction with cellulose. Alkaline materials, such as soda ash, borax, sodium acetate (salts of a strong base and a weak acid) are also effective as catalysts.

Cellulosic material is impregnated with the solution or dispersion by immersion, dipping, or spraying, preferably followed by passage through squeeze rolls. Cellulosic fabrics may also be printed with a solution or paste, thus producing local effects. The impregnated material is dried at room temperature or above and heated to a temperature preferably between 90° C. and 130° C. In this temperature range the reaction between cellulose and the aminomethylene aminotriazine takes place in a short time with the triazine nucleus becoming chemically combined with the cellulose. Somewhat lower temperatures and higher temperatures are also effective. Drying and heating may constitute one continuous operation. After the step involving heating, the treated material may be washed to remove unreacted material, or decomposition products from the reacted aminomethylene amino-1,3,5-triazine.

The "animalizing" of the cellulose may be combined with a sizing operation resulting in simultaneous fixation of the size as disclosed in our copending application Serial No. 300,655 filed Oct. 21, 1938, which on Nov. 10, 1942, issued as U. S. Patent No. 2,301,509 and in "animalizing" of the cellulose. In the preferred procedure the operation of dyeing follows the modifying of the cellulose. The treated cellulose is receptive to acid and basic dyes and to any other dyestuffs which are normally used only on wool or silk. The aminomethylene amino-1,3,5-triazines are also useful in conjunction with resin-finishing of fabrics, serving as softening agents when the triazine group carries a hydrocarbon substituent of twelve or more carbon atoms.

Typical treatments of various cellulosic materials are shown in the following examples—

**Example 1.**—A bleached cotton fabric was coated with a composition containing 12.5% of tris(dimethylaminomethyl) melamine, 3.5% of water-soluble hydroxyethyl cellulose, 1% acetic acid and 83% of water. It was dried, heated one-half hour at 130° C., and washed. It was then dyed one-half hour in a boiling 5% solution of Pontacyl Carmine 6B containing 1% of acetic

acid and took on a medium dark red shade, which was fast to washing.

**Example 2.**—Cotton fabric was dipped through a solution containing 12% of the bis-(dimethylaminomethyl) derivative of thioammeline and 0.5% of acetic acid in water. It was squeezed and dried, then heated one-half hour at 120° C., and finally washed. A sample dyed as in Example 1 acquired a dark color, which was fast to 10 washing.

**Example 3.**—Cotton yarn was dipped through an aqueous solution containing 10% of acetic acid and 25% of a dimethylaminomethyl derivative of 1-cyano-2-amino-4,6-dimethyl tetrahydrotriazine. It was dried, heated twenty minutes at 130° C., and washed. On dyeing as in Example 1, a medium shade of color was obtained which was fast to washing.

**Example 4.**—A viscose rayon fabric was dipped 20 through a paste comprising 12.5 parts of the bis-(dimethylaminomethyl) derivative of melamine, 4% of potato starch, 5% of acetic acid, and 78.5% of water. It was then dried, heated at 130° C. for twenty minutes, and washed. The 25 dyeing operation, performed as in Example 1, gave a deep color which was retained on washing.

**Example 5.**—Cellulose acetate fabric was dipped through an aqueous solution containing 30 25% of the tris-(dimethylaminomethyl) derivative of dibutyl ammeline. It was then dried, heated at 130° C. for twenty minutes, and dyed at the boil with Pontacyl Carmine 6B. The cellulose acetate was dyed to a medium red shade 35 which was fast to washing.

**Example 6.**—Cotton fabric was dipped through a 12% solution of dimethylaminomethyl ammeline acidified with acetic acid and was squeezed. It was dried, baked one-half hour at 40 130° C., and washed. Upon immersion at 95° C. for twenty minutes in a 0.5% fuchsin solution, it acquired a deep wine-red color, resistant to washing.

**Example 7.**—Cotton fabric was dipped through 45 a paste comprising four parts of a 7% aqueous solution of hydroxyethyl cellulose and 1 part of bis-(dimethylaminomethyl) melamine hydrochloride. After removing the excess with a squeeze roll, the fabric was heated one-half hour 50 at 130° C. and washed. Treatment of the stiffened fabric with fuchsin as in Example 6 gave a wine-red color, which was permanent.

**Example 8.**—Linen fabric was treated according to Example 6. With the same basic dye, it 55 gave a medium wine-red shade, resistant to washing.

**Example 9.**—Cotton sheeting was run through an aqueous solution containing 5% of bis-(dimethylaminomethyl) diarachidyl ammeline and 60 0.25% of sodium carbonate. The wet cloth was placed in an oven and baked one-half hour at 140° C. The resulting fabric was very resistant to wetting and this property was not materially affected by washing. A pleasing fullness and 65 softness was also imparted to the sheeting.

**Example 10.**—Example 9 was repeated using bis-dimethylaminomethyl distearyl ammeline. The results were similar, a high degree of resistance to wetting and of softness being obtained.

**Example 11.**—Cotton sheeting was coated with a paste containing 5% of dimethylaminomethylene distearyl ammeline and 0.25% of sodium carbonate. It was baked one-half hour at 140° C. A water-repellent finish was obtained. The hand was full, soft, with a dry, wax-like feel.

*Example 12.*—A rayon pile fabric was impregnated with a 2% solution of bis-dimethylamino-methyl distearyl ammeline. It was baked one-half hour at 125° C. A soft hand was obtained and resistance to wetting.

*Example 13.*—A piece of 80 x 80, 4-yard, 36-inch cotton sheeting was fastened in a rigid frame and treated under tension with a 15% aqueous solution of tris(dimethylaminomethyl) melamine hydrochloride. It was placed in an oven without drying and held at 130° C. for twenty minutes. After a soap wash at 140° F. for one-half hour, it had shrunk 2.5% in the warp-wise dimension. A control shrank 5.0%.

We claim:

1. A method for preparing nitrogenous cellulose derivatives on water-insoluble cellulosic materials in the form of fabrics, yarns, fibers, battings, sheets, and strips which comprises treating the cellulosic material with a solution of a condensation product of an amino-1,3,5-triazine and at least molecular proportions of formaldehyde and dimethylamine, and heating the treated material to a temperature between about 90° and about 140° C.

2. A method for preparing nitrogenous cellulose derivatives on water-insoluble cellulosic materials in the form of fabrics, yarns, fibers, battings, sheets, and strips which comprises treating the cellulosic material with a solution of a condensate of distearyl ammeline with at least molecular proportions each of formaldehyde and dimethylamine, and subsequently heating the treated material to a temperature between about 90° and about 140° C.

35

3. A method for preparing nitrogenous cellulose derivatives on water-insoluble cellulosic materials in the form of fabrics, yarns, fibers, battings, sheets, and strips which comprises
  - 5 treating the cellulosic material with a solution of a condensate of melamine and at least molecular proportions each of formaldehyde and dimethylamine, and subsequently heating the treated material to a temperature between about 90° and about 140° C.
  - 10 4. A method for preparing nitrogenous derivatives on fabrics, yarns, fibers, battings, sheets, and strips composed of water-insoluble regenerated cellulose which comprises treating said regenerated cellulose with a solution of a condensation product of an amino-1,3,5-triazine with at least molecular proportions each of formaldehyde and dimethylamine, and subsequently heating the thus treated cellulose to a temperature between about 90° and about 140° C.
  - 15 5. Cellulosic textile fabric carrying a complex reaction product formed by heating to a temperature between about 90° C. and about 140° C. cellulose and a condensation product of melamine with at least molecular proportions each of formaldehyde and dimethylamine.
  - 20 6. A cellulosic textile fabric carrying a complex reaction product formed by heating to a temperature between about 90° C. and about 140° C. cellulose and a condensate of distearyl ammeline with at least molecular proportions each of formaldehyde and dimethylamine.
  - 25

LOUIS H. BOCK  
ALVA L. HOUK.